

# UNITED STATES PATENT OFFICE.

RUDGYARD I. SMITH, OF WASHINGTON, DISTRICT OF COLUMBIA, ASSIGNEE OF ONE-FOURTH TO MAUD H. SMITH, OF TAKOMA PARK, DISTRICT OF COLUMBIA, AND ONE-FOURTH TO WILLSON H. KNIGHT, OF TAKOMA PARK, MARYLAND.

## PROCESS OF PRESERVING WOOD.

1,129,430.

Specification of Letters Patent. Patented Feb. 23, 1915.

No Drawing.

Application filed November 7, 1913. Serial No. 709,282.

*To all whom it may concern:*

Be it known that I, RUDGYARD I. SMITH, a citizen of the United States, residing at Washington, in the District of Columbia, have invented certain new and useful Improvements in Processes of Preserving Wood, of which the following is a specification:

My invention has to do with the preservation of wood by the saturation or impregnation of the wood with certain chemicals. To this end I employ a process which is not only economical in the material to be used and capable of being carried out with an inexpensive equipment, but produces results not attainable with processes heretofore employed.

Another object of my invention is to employ certain chemicals as above stated which when used as hereinafter described, will cause a certain reaction to take place in the wood which will result in the precipitation of an insoluble precipitate throughout the wood. Heretofore it has been difficult to get sufficient penetration for reasons that preservatives that are satisfactory as sterilizers will not enter freely into the pores of the wood or thoroughly attack the active fermenting contents of the wood.

One feature of my invention therefore consists in treating the wood, first, with a solution that enters freely into the innermost pores of the wood, and, then with a disinfecting agent which follows freely wherever the first agent has penetrated, and the thoroughness of the process is thereby insured. For the first agent I preferably select a solution of an antiseptic nature to assist in disinfecting the fermenting properties of the wood, and this first agent is preferably a solvent of the fermenting content. Heretofore for the sake of economy, solutions of salts in water have been employed for purposes of preserving wood, but as heretofore practised, such solutions have been too readily washed out to develop any lasting effect.

Another feature of my invention consists in employing for both the first and subsequent solutions, soluble salt in water, so that economy is attained, but I select such salts that will enter and penetrate the innermost pores of the wood and remain indefinitely.

To obtain the best results I have found it necessary to subject the wood to a hot solution of the first agent, also to treat the wood with the finishing agent without undue loss of time after it has been removed from the first solution.

In carrying out the invention I prefer to employ a solution of ordinary commercial copperas or iron sulfate for the first solution, and a solution of ordinary blue vitriol or copper sulfate for the subsequent treatment. I have found in practice that a solution of iron sulfate in the proportions of about one pound of iron sulfate to 2 gallons of water, and a solution of copper sulfate in the proportions of one pound of copper sulfate to about 2 gallons of water will effectively produce the desired results if applied in accordance with my invention, viz., by first soaking the wood in the first solution for from 12 to 24 hours according to the character of the wood and then soaking the wood thus saturated in the second solution for from 12 to 24 hours. I have found by experiment extending over months, and even years, that wood thus treated will withstand decay and be less liable to split. I have also found that wood treated in accordance with my invention will not deteriorate when placed in water or subjected to different atmospheric conditions. Furthermore, I have found that the original elasticity or resiliency of the wood is not destroyed by this treatment. My treatment or process may be applied to either the seasoned or unseasoned wood with the same valuable results.

While I know from actual tests which I have made that a certain chemical reaction takes place in the wood treated by my process, I have thus far been unable to determine just what this reaction is.

I claim:

The process of treating wood for preserving it which consists in first soaking it in a solution of sulfate of iron and then subjecting it to a solution of sulfate of copper.

In testimony whereof I affix my signature in presence of two witnesses.

RUDGYARD I. SMITH.

Witnesses:

EVA V. LEITH,  
DOROTHY S. KNIGHT.